

## UNITED STATES PATENT OFFICE

2,096,201

## ALLOY

Donald W. Randolph, Flint, Mich., assignor to  
General Motors Corporation, a corporation of  
Delaware

No Drawing. Application August 18, 1934, Se-  
rial No. 740,537. In Germany and Canada  
April 16, 1934

2 Claims. (Cl. 75—159)

This is a continuation in part of my prior application Serial No. 667,502, filed April 22, 1933.

This invention has to do with alloys containing barium, a material of low work function, readily giving off electrons when energy is applied to it, such application of energy usually being in the form of either heat or electricity as in the conventional types of radio tubes. The invention also has to do with electron emitters made of such 10 alloys.

In the prior application of Hugh S. Cooper, Serial No. 655,138, filed February 3, 1933, there is disclosed a method of making alloys of an alkaline earth metal, preferably barium, and nickel, 15 which consists in employing a proportion of copper in the melt to hold the barium in solution. There are also disclosed in said application certain new alloys of the above description and electron emitters made of such new compositions.

As a result of independent but later work I likewise discovered the usefulness of copper in increasing the barium content of alloys containing nickel and barium and in addition have discovered that the addition of chromium to the 25 melts produces finer grained alloys and gives to emitters made of such alloys advantages not possessed when chromium is omitted. Thus I have found that radio tube filaments made of nickel, barium, copper, and chromium alloys may be 30 operated for long periods without substantial deterioration at temperatures at which filaments of the same composition but with chromium omitted would rapidly deteriorate. Chromium appears to definitely inhibit evaporation of ba- 35 rium and so preserves the emitting surface. I also found that electrodes made of the same alloy when used for arc or spark discharge last many times longer than electrodes made of the same alloys lacking chromium. The addition of chro- 40 mium results in metal of finer grain size under the same cooling and pouring conditions and it may be that this characteristic of the chromium containing alloys is related in some way to the longer life of the electrodes.

I have prepared the described alloys by the method disclosed in my prior Patent No. 1,919,- 479, granted July 25, 1933, that is, by melting the base metal or metals, wrapping the barium addition in foil or coating it to prevent oxidation and 45 thereafter inserting it in the melt, holding the melt for a short time at an elevated temperature to permit thorough alloying and thereafter pouring. However while alloys of the desired high barium content could be made by this process, if 50 the barium content was over about .25% the alloys were hard and brittle and could not be satisfactorily rolled or otherwise worked. Such alloys were found to be high in gas content and so an effort was made to eliminate gases there- 55 from.

Attempts were accordingly made to eliminate gas by covering the melt with an atmosphere of  $\text{CO}_2$  or other inert gas but unsatisfactory results were obtained. Following this a number of trials were made with slags on the melt to exclude air, 5 the barium being added through holes made in the slag. Here difficulty was encountered in obtaining a slag sufficiently sticky to form a gas tight seal. Best results were obtained with the use of a glass of the following composition, this 10 glass being sticky over the range of temperature used in melting:

|                         | Per cent |
|-------------------------|----------|
| $\text{BaO}$            | 32.6     |
| $\text{B}_2\text{O}_3$  | 8.7 15   |
| $\text{K}_2\text{O}$    | 5.4      |
| $\text{Al}_2\text{O}_3$ | 13.1     |
| $\text{SiO}_2$          | 40.2     |

The gas content of the metal was reduced by 20 superheating under the slag and continuing this until gas ceased to bubble through the slag. Thereafter the melt was cooled to pouring temperature, about .1% magnesium was added as a deoxidizer, followed by the addition of barium in 25 the manner described. The melt was then held for a time varying from 30 seconds to two minutes depending on the amount of barium added, a longer time being required with the higher barium contents. The slag was then removed and 30 the metal poured into cold iron molds.

While better and more workable alloys were obtained by this process difficulty was nevertheless encountered because of the tendency of the barium to react with the constituents of the slag 35 producing oxide inclusions in the melt. Far more satisfactory results have been obtained by melting the base metals under vacuum, preferably in an induction furnace, and following the melting with further heat treatment under vacuum at 40 temperatures several hundred degrees above the melting point to further reduce the gas content. When the melt has been sufficiently degassed, an inert gas is introduced into the furnace surrounding the melt and the barium is then introduced into the melt through the inert atmosphere. 45 After allowing a sufficient time for thorough alloying, the furnace, which is preferably mounted on pivots after the manner of a Bessemer converter, is inverted and the melt is poured into a mold enclosed in the furnace chamber and, of course, immersed in the same inert atmosphere. With this procedure the gas initially in the melt 50 is first removed and all the operations thereafter are so conducted that oxidation and absorption of gases is almost entirely avoided. This method is to be covered in a patent application about 55 to be filed.

Employing the method last described it has proven possible to produce alloys both of nickel, 60

5 barium, copper and of nickel, barium, copper and chromium of widely varying compositions that are as ductile as is desirable for any practical purposes. Thus such alloys have been drawn into very fine wires or filaments and have been rolled into very fine ribbons and other shapes.

10 I have made by the methods described, alloys of nickel, barium and copper falling within the following range:

|        | Percent      |
|--------|--------------|
| Nickel | 95 to 5      |
| Copper | 5 to 95      |
| Barium | 0.25 to 10.5 |

15 In general the higher the copper content, the higher the amount of barium that can be alloyed. To these alloys we have usually added a small amount of magnesium, approximately 0.1%, as a deoxidizer, but this may be omitted if desired for barium itself may serve the same purpose. Other known deoxidizers such as calcium are indicated as suitable for this purpose.

20 Manganese may likewise be added to the melt, but I have found it somewhat undesirable because of its high gas content. Other additions 25 in the nature of diluents will readily occur to those skilled in metallurgy.

25 I have also used strontium in place of barium, and, while successful in securing homogeneous 30 alloys of high strontium content, the emission has proven somewhat disappointing as compared to barium. For example, an alloy containing 35 .8% strontium, 25% copper and the balance nickel was found to give but one-tenth of the electronic emission that was obtained from an alloy containing .8% barium, 25% copper and the balance nickel.

40 I have added varying amounts of chromium to the alloys described above in order to secure the advantage of the evaporation-inhibiting effect of chromium on the barium in the alloy as well as increased resistance to corrosion. The workability of the alloy is decreased by the addition of chromium. Such alloys may be made in the manner above described within the following 45 range of ingredients:

|             | Percent      |
|-------------|--------------|
| Nickel      | 5 to 95      |
| Copper      | 5 to 95      |
| Barium      | 0.25 to 10.5 |
| 50 Chromium | 0.1 to 25    |

To these alloys the auxiliary materials mentioned above may likewise be added if desired.

No difficulty is encountered in the melting procedure due to the addition of chromium although more gas is given off. The addition of chromium does not greatly affect the alloying of barium. The chromium practically all alloys with the 5 nickel, as copper-chromium alloys can only be made with great difficulty.

The described alloys have been made into filaments for radio tubes and into electrodes for gaseous discharge tubes such as are described and 10 claimed in the prior application of Duffendack and Wolfe, Serial No. 716,972, filed March 23, 1934. Where the alloy is used as an electrode in such tubes a chromium content of from  $\frac{1}{2}$  to 2% has been found to be sufficient to give the 15 desired results.

In order to obtain the high rate of emission that is desired, filaments made of the described alloys are preferably oxidized and then activated by heating in a vacuum as described and claimed 20 in the patent of Duffendack and Wolfe No. 1,909,-916, granted May 16, 1933. In the testing of such emitters it has been found that those containing chromium can be operated at higher temperatures since the chromium definitely inhibits 25 evaporation and so prevents destruction of the emitting surface. In the case of such emitters a chromium content of from 1 to 5% permits operation of the emitter at a temperature higher than in the absence of chromium. In some cases 30 the emitter may be operated approximately 100° C. hotter without loss by evaporation or decrease in emission due to breaking down in the emitting surface. As a consequence a somewhat increased output is obtainable from an emitter of a given 35 size.

It is possible by varying the chromium content to control the electrical resistance of the alloy and this is of value in cases where an emitter is a directly heated filament as the resistance of the 40 filament may be adjusted to a wide range of values without changing its size.

I claim:

1. An alloy characterized by ready emission of electrons consisting of from .25% to 10.5% 45 barium, from .1% to 25% chromium, from 5% to 95% copper and from 5% to 95% nickel.

2. An alloy characterized by ready emission of electrons and durability under emitting conditions consisting of from .25% to 10.5% barium, 50 from .5 to 5% chromium, from 5% to 95% copper and from 5% to 95% nickel.

DONALD W. RANDOLPH.